

Patented Dec. 27, 1927.

1,653,630

## UNITED STATES PATENT OFFICE.

EDWARD KIAM, OF NEW YORK, N. Y., ASSIGNOR OF ONE-HALF TO MATTHEW G. COLLINS, OF NEW YORK, N. Y.

### ALLOY.

No Drawing. Application filed February 25, 1922, Serial No. 539,098. Renewed May 19, 1927.

This invention relates to alloys.

An object of this invention is to provide a non-ferrous alloy having metallic properties generally but which is free from substantial attack by sulphuric, nitric and hydrochloric acids, ammonia chloride, acetic acid, chlorine, ammonia, mine waters, alkalies, also free from attack by sulphurous fumes and the gases evolved in the production, refining and manufacturing of oils, and also free from attack by common hypo-chlorites and hypo-sulphites.

Pursuant to my invention, the alloy comprises nickel, tungsten, chromium, manganese and magnesium, the nickel content being of relatively high proportion relative to tungsten and chromium; the manganese content being less than the tungsten or chromium content, and the magnesium content of relatively low proportion relative to tungsten and chromium.

In the various forms of the invention, the nickel content varies within the range of 30 to 65 per cent, the tungsten content from 15 to 40 per cent; the chromium content from 15 to 30 per cent, the manganese content from 1 to 8 per cent and the magnesium from 5 to one-half of one per cent. The nickel content preferably exceeds the sum of the content of tungsten and the content of chromium.

The nickel content of the alloy is added in the form of a nickel containing ingredient or ingredients free from sulphur.

The alloy is formed by taking ingredients embodying the above metals respectively in metallic form and heating the mixture, whereupon the metal contents of nickel tungsten, chromium, manganese and magnesium are merged into an alloy.

The most preferred method of forming the alloy is by taking the commercially pure metals in the proportions as above named and melting the same to obtain an intermixed molten mass, which upon cooling

yields the solid alloy of the above constituency.

The most preferred form of the alloy consists of a nickel content greater than the sum of the tungsten and chromium contents, the tungsten and chromium contents being substantially equivalent; the manganese content being less than each of the tungsten and chromium contents and the magnesium content being less than the manganese content.

The alloy possesses metallic properties, but is substantially free from attack by sulphuric acid, or by nitric acid, or by hydrochloric acid. The alloy is also free from attack by sulphurous fumes, lime water, chlorine and the gases created in the distilling and refining of crude petroleum and other mineral oils. The alloy is also free from attack by calcium and other common commercial hypo-chlorites and by sodium and other common commercial hyposulphites.

I claim:

1. An alloy consisting of nickel in the proportion of from thirty percent to sixty-five percent; of tungsten in the proportion of from fifteen percent to forty percent; of chromium in the proportion of from fifteen percent to thirty percent; of manganese in the proportion of from one percent to eight percent; and of magnesium in the proportion of from five percent to one-half of one percent.

2. An alloy consisting of nickel in the proportion of from thirty percent to sixty-five percent; of tungsten and chromium in substantially equivalent proportion to one another; of manganese in the proportion of from one percent to eight percent; and of magnesium in the proportion of from five percent to one-half percent, the aforesaid proportions totalling one hundred percent.

In testimony whereof I have signed this specification this 24th day of February, 1922.

EDWARD KIAM.